# EUROPEAN PATENT APPLICATION

(11) **EP 4 617 345 A1**
(43) Date of publication of application: **17.09.2025**
(21) Application number: 24890326.2
(22) Date of filing: 19.09.2024
(51) Int. Cl.: C10L 1/12, C10L 3/00, C10L 9/10, F23K 5/08, F23K 5/00, F23K 1/00

(54) **METHOD FOR PROMOTING COMBUSTION OF COMBUSTIBLE MATERIAL, IMPROVING POWER OUTPUT OF COMBUSTION DEVICE AND PROLONGING SERVICE LIFE OF COMBUSTION DEVICE**

(30) Priority: 16.11.2023 CN 202311528556
(71) Applicant: Qingdao Hengnengda Energy Technologies Co., Ltd., Qingdao, Shandong 266000 (CN)
(72) Inventor: ZHANG, Yongheng, Qingdao, Shandong 266000 (CN)
(74) Representative: ABG Intellectual Property Law, S.L.
(86) International application number: PCT/CN2024/119696
(87) International publication number: WO 2025/102967

(57) **Abstract**

A method for promoting the combustion of a combustible material, improving the power output of a combustion device and prolonging the service life of the combustion device by adding an alkali metal element and/or an alkaline earth metal element into the combustible material, relating to the technical field of combustion supporting. The method is applicable to various combustible materials and various combustion devices. A combustion device, and a fuel for promoting the combustion of a combustible material, improving the power output of a combustion device and prolonging the service life of the combustion device, respectively comprising a combustion device, and a fuel for nuclear fusion and nuclear fission. The method can enable all kinds of combustion devices to be reliably started and efficiently and safely work in any environment.

## Description

### Technical Field

This invention is about combustion promotion technology, which relates to a method to promote combustion of combustible and enhance power output and usage life of combustion equipment. This invention discloses to promote combustion of combustible and enhance power output and usage life of combustion equipment thereof by adding alkali metal element and/or alkaline earth metal element into the combustible. This invention discloses a fuel and a combustion equipment including the fuel and reactor for nuclear fusion or nuclear fission to promote combustion of combustible and enhance power output and usage life of combustion equipment. Importantly, the disclosed fuel or combustion equipment can prevent explosive combustion. By using the method, the combustion efficiency of combustible, power output and usage life of combustion equipment can be significantly enhanced, and the safety of combustion process can be improved significantly.

### Background Technology

The existing technology believes that a combustion is a violent, luminous, and exothermic chemical reaction that occurs between the combustible and combustion supporting material. The characteristic of combustion supporting material is its ability to support the combustion. When a piece of paper burns in oxygen, the oxygen has a combustion supporting property. When a piece of magnesium burns in carbon dioxide, the carbon dioxide has combustion supporting property. The combustion supporting material does not have a combustibility, and the combustible does not have a combustion supporting property. The combustible and combustion supporting material are interdependent. Both combustible and combustion supporting material are necessary for combustion.

The existing technology believes that the combustion supporting material can increase the combustion performance and improve combustion efficiency, and they are generally considered as oxidants. For example, the oxygen is used as the oxidant in the combustion of daily life. The combustion supporting materials can also be added into various fuels for various combustion equipment such as industrial boiler, car and ship engine, jet engine, or rocket engine, or be added into explosive and gunpowder, etc.

It is believed in prior arts that the combustion efficiency, power output, noise, vibration and usage life are only related to combustion process. In the past 100 years, the improvement of combustion efficiency, power output, noise and vibration, and usage life of combustion equipment is usually based on the design of combustion equipment structure. The promotion of the combustion process is usually achieved by adding the oxidants without considering the interaction between the fuel and combustion equipment during the combustion process. However, the improvement of combustion, power output and usage life of the combustion equipment is not significant.

### Summary of Invention

In order to solve the aforementioned problems, this invention discloses a method to promote the combustion of combustible and enhance power output and prolong usage life of combustion equipment. The method disclosed in this invention is completely different from the principles of existing combustion promotion technologies. In this method, the alkali metal element and/or alkaline earth metal element is added into the combustible material to promote the formation of plasma to promote the combustion of combustible and enhance power output and usage life of combustion equipment.

In order to achieve above technical purpose, this invention provides following technical solutions:
A method for promoting combustion of combustible and enhancing power output and usage life of combustion equipment by adding alkali metal element and/or alkaline earth metal element into the combustible. The matter state of combustible comprises at least one of gas, liquid and solid. The alkali metal element comprises one or more of Li, Na, K, Rb, Cs and Fr, and the alkaline earth metal element comprises one or more of Be, Mg, Ca, Sr, Ba and Ra.

The method disclosed in this invention is applicable to all combustible.

The combustible comprises one or more of carbon, carbon containing organic matter, hydrogen, deuterium, tritium, ammonia, metal, sulfur and phosphorus.

The disclosed technology is applicable to all combustion equipment, for example, gasoline engine, diesel engine, internal combustion engine, external combustion engine, piston engine, piston engine using ammonia mixed fuel, piston engine using hydrogen mixed fuel, turbofan engine, turbojet engine, rocket engine, gas turbine, mixed fuel turbine, boiler, nuclear fusion reactor, nuclear fission reactor, fuel cell, warmer, oven, thermoelectric converter, combustion refrigerator.

The alkali metal element and/or alkaline earth metal element is added into the combustible by a form comprising at least one of atom, ion and plasma.

The alkali metal element and/or alkaline earth metal element is added into the combustible by any matter containing alkali metal element and/or alkaline earth metal element.

The matter containing alkali metal element and/or alkaline earth metal element comprises one or more of elementary substance, alloy, compound or composition of all alkali metal element and/or alkaline earth metal element, and the state of matter containing alkali metal element and/or alkaline earth metal element comprises gas, liquid, solid or plasma.

Preferably, the addition amount of alkali metal element and/or alkaline earth metal element is 0wt%-100000.9999999999999999wt% of mass of combustible, and not to be 0.

Preferably, the addition amount of the alkali metal element and/or alkaline earth metal element is Owt% - 90.9999999999999999wt% of mass of combustible, and not to be 0.

The approach for adding alkali metal element and/or alkaline earth metal element into the combustible comprises at least one of approach 1, 2, 3 or 4.

The approach 1 comprise: to add the matter containing alkali metal element and/or alkaline earth metal element into the combustible by melting, electric sparking, plasmazing, mixing, ball milling, or crushing; or to mix the matter containing alkali metal element and/or alkaline earth metal element with noncombustible followed by adding the mixture into the combustible.

The approach 2 comprises: to dissolve the matter containing alkali metal element and/or alkaline earth metal element into the combustible.

The approach 3 comprises: to dissolve the matter containing alkali metal element and/or alkaline earth metal element into a solvent to obtain a solution, or suspension or paste followed by adding it into the combustible.

The approach 4 comprises: to add the matter containing alkali metal element and/or alkaline earth metal element into a part of combustion equipment. The alkali metal element or alkaline earth metal element in the part will react with the combustible or noncombustible forming a chemical species containing alkali metal element and/or alkaline earth metal element, which will be added into the combustible.

In approach 4, the part comprises one or more of combustion chamber, or piston, piston connecting rod, cylinder liner, rotor, blade, lighter, spark plug, gear, bearing, bolt, nut inside combustion chamber, pipeline or tank of oil, fuel or combustion supporting material.

In approach 4, the part of combustion equipment is made of material containing alkali metal element and/or alkaline earth metal element. The material containing alkali metal element and/or alkaline earth metal element comprise one or more of polymer, ceramics or metal. The content of alkali metal element and/or alkaline earth metal element in the material containing alkali metal element and/or alkaline earth metal element is 0wt%-99.990000000000wt%, and not to be 0.

The polymer comprises rubber. The metal comprises elementary substance of metal or alloy. The content of alkali metal element and/or alkaline earth metal element in alloy is 0.00000000001wt%-99.99wt%.

This invention further provides a combustion equipment. During combustion process, the alkali metal element and/or alkaline earth metal element react with the combustible forming a carbon-containing material on surface of combustion equipment, and the carbon-containing material is the matter containing alkali metal element and/or alkaline earth metal element. Therefore, in this invention, the part of combustion equipment has a dent, protrusion or hole, so as to produce different matters containing alkali metal element and/or alkaline earth metal element. During combustion process, the dent, protrusion or hole will add different matters containing alkali metal element and/or alkaline earth metal element to different spaces of combustion chamber, so as to adjust combustion state inside combustion chamber and realize the control of combustion process. Additionally, the matter containing alkali metal element and/or alkaline earth metal element inside the dent or hole acts as a storage of alkali metal element and/or alkaline earth metal element during combustion process to prevent the deletion or content fluctuation of alkali metal element and/or alkaline earth metal element during combustion process. The part comprises one or more of combustion chamber, piston, piston connecting rod, cylinder liner, nozzle, spark plug, rotor, blade, bearing, bearing seat, bolt or nut inside combustion chamber.

The maximum cross-sectional area of the orifice of through-hole or dent, or base of protrusion of the part is from 0.01 square nanometers to 1 square meters. The depth of dent or height of protrusion is from 0.1 nm to 100 mm. The dent or protrusion is any geometry. The part comprises one or more of combustion chamber, or parts inside combustion chamber.

At the same time, according to this invention, the part or some parts of combustion equipment are further produced by the material containing alkali metal element and/or alkaline earth metal element. The content of alkali metal element and/or alkaline earth metal element of the material containing alkali metal element and/or alkaline earth metal element is from 0wt%-99.990000000000wt%, and not to be 0. The material containing alkali metal element and/or alkaline earth metal element comprises polymer, ceramics or metal. The combustion equipment comprises any kind of combustion equipment. The combustion equipment can promote the combustion of combustible, has higher power output and longer usage life and higher mechanical reliability.

According to above control theory of combustion, this invention discloses a piston engine. The piston engine is characterized by having dent on inner surface of cylinder, or dent and/or protrusion on outer surface of cylinder. The dent or protrusion is any geometry. There is or is not protrusion in dent. The arrangement of dent or protrusion is regular or irregular.

The cross-sectional area of orifice of dent or base of protrusion is from 0.01 square nanometers to 0.03 square meters. The depth of dent or height of protrusion is from 0.1 nm to 100 mm.

There is groove or blind hole on inner surface and/or outer surface of cylinder. The width of groove or diameter of blind hole is from 0.001 µm to 10 mm. The depth of groove or blind hole is from 0.001 µm to 10 mm.

Further, the part or some parts of disclosed piston engine are produced by material containing alkali metal element and/or alkaline earth metal element. The content of alkali metal element and/or alkaline earth metal element in the material containing alkali metal element and/or alkaline earth metal element is from 0wt%-99.990000000000wt%, and not to be 0. The material containing alkali metal element and/or alkaline earth metal element comprises polymer, metal or ceramics. The part comprises one or more of the combustion chambers, piston, piston connecting rod, cylinder liner, nozzle, spark plug, bolt, nut inside combustion chamber, tank or pipeline of oil, fuel, or combustion supporting material.

Further, the disclosed piston engine comprises or does not comprises liquid cooling system, the piston engine uses the combustible comprising one or more of gasoline, diesel, bio-diesel, plant oil, animal oil, bio-ethanol, bio-methanol, ethanol, methanol, ammonia, hydrogen, natural gas, acetylene, liquidized petroleum gas, or polymer-based or plant-based carbon-containing organic matter.

There is a carbon-containing material formed on part surface of combustion equipment during the combustion process due to the combustible containing alkali metal element and/or alkaline earth metal element. The thickness of the carbon-containing material is from 0.1 nm to 1 mm. The surface of carbon-containing material has any structure and macroscopic morphology. The carbon-containing material acts as a buffer storage of alkali metal element and/or alkaline earth metal element, and has one or more functions of lubrication, sealing, thermal conductivity, thermal insulation, high and low temperature resistance, wear resistance, thermal shock resistance, corrosion resistance, explosive combustion resistance, or surface defect repairment of combustion equipment. Therefore, the combustion equipment or fuel disclosed by this invention can make combustion equipment having excellent characteristics comprising lubrication, sealing, thermal conductivity, thermal insulation, high and low temperature resistance, wear resistance, thermal shock resistance, corrosive resistance, explosive combustion resistance, thermal fatigue resistance, or surface defect repairment of combustion equipment. Therefore, the combustion equipment can withstand a higher combustion temperature and gas pressure, and can be without liquid cooling system or external forced lubrication system.

Further, the method of this invention can intake more air or other kinds of combustion supporting gas, hence, the combustion equipment can use a high pressure intake system to enhance the amount of produced gas or cylinder pressure to improve the power output of piston engine.

Specially noted, the piston engine disclosed in this invention comprise the piston engine using one of all kind combustible, for example, gasoline engine, diesel engine, internal combustion engine, ammonia mixed fuel engine, hydrogen mixed fuel engine, or mixed fuel piston engine.

This invention also provides a fuel which can enhance the power output and usage life of combustion equipment. The fuel comprises combustible and alkali metal element and/or alkaline earth metal element. Preferably, the addition amount of alkali metal element and/or alkaline earth metal element is 0wt%-100000.9999999999999999wt% of mass of the combustible, and not to be 0.

Preferably, the mass of alkali metal element and/or alkaline earth metal element is 0wt%-90.9999999999999999wt% of mass of the combustible, and not to be 0.

The fuel provided by this invention is applicable to all kind of combustion equipment, and can prevent explosive combustion and promote the combustion of combustible and enhance the power output and prolong usage life of combustion equipment, as well as make the combustion equipment work safely. The examples of the fuel comprise anti-explosive combustion fuel, internal combustion engine fuel, external combustion engine fuel, piston engine fuel, mixed fuel engine fuel, mixed fuel, turbofan engine fuel, turbojet engine fuel, gas turbine fuel, boiler fuel, fuel cell fuel, nuclear fusion fuel, nuclear fission fuel, warmer fuel, oven fuel, thermoelectric converter fuel and combustion refrigeration fuel.

This invention also provides a high efficiency energy conversion system, which comprises the fuel and combustion equipment. The fuel is the above fuel. The combustion equipment is the above combustion equipment. The high efficiency energy conversion system can start, work, prevent explosive combustion, output higher power and have longer usage life at any environment.

In order to further improve the combustion efficiency of combustible, the high efficiency energy conversion system further includes other energy conversion equipment connected to combustion equipment. The other energy conversion equipment comprises one or more of refrigeration equipment, hot water boiler, steam boiler, industrial kiln, industrial oven, thermoelectric converter, or generator driven by steam boiler.

This invention provides a method for promoting combustion of combustible and enhancing power output and usage life of combustion equipment by adding alkali metal element and/or alkaline earth metal element into the combustible. The inventor Professor Dr. Yongheng ZHANG (Professor Dr. Yongheng ZHANG is the lawful representative, president, and manager of Qingdao Hengnengda Energy Technologies Co., Ltd., China, he has PhD, MSc and BSc in material engineering and is the professor of materials science 2004.) has found that the combustion of combustible must have the process of plasma formation. The carbon-containing organic matter must be lighted for combustion. (For example, the match lights a piece of paper, the electrical lighter lights the natural gas, the spark plug lights the gasoline inside cylinder.) These sparks comprise plasma. There must be alkali metal element and/or alkaline earth metal element making the combustible generating more plasma. These plasmas will continue to ignite more combustible and form more plasma to let the combustion process continue until complete burn out of the combustible. If there is no alkali metal element and/or alkaline earth metal element in the combustible or environment, or if the environmental temperature is not over a critical temperature, the combustion cannot be ignited and proceeds. Similarly, other types of combustibles such as hydrogen, deuterium, tritium, ammonia, sulfur, phosphorus, or metal also require a plasma to initiate and keep their combustion. The formation of plasma must involve alkali metal element and/or alkaline earth metal element. This is to say that the alkali metal element and/or alkaline earth metal element is essential element for plasma formation.

Based on the combustion principle of combustible disclosed by the inventor, the alkali metal element and/or alkaline earth metal element is added into the combustible to initiate the combustion, promote the formation of more plasma at one time, thereby promoting the combustion of the combustible. By controlling the amount of alkali metal element and/or alkaline earth metal element in the combustible, the combustion process, combustion characteristics (such as combustion color, temperature distribution, combustion rate, airflow speed and direction) can be controlled. More importantly, the technology of the present invention is applicable to all types and forms of combustible and all kind of combustion equipment.

During the combustion process, the alkali metal element and/or alkaline earth metal element reacts with the surface layer of the combustion equipment, damaging the surface layer of the combustion equipment and generating heat. When the surface layer of the combustion equipment cannot be rebuilt, the temperature of the combustion equipment and environment will continue to rise until the combustion chamber is melted. When the destroy and rebuild of the surface layer of the combustion equipment reaches an equilibrium, the temperature of the combustion equipment reaches constant and the combustion equipment is heated. And at the same time, the environmental temperature is heated. During the combustion process, the destroy and rebuild of the surface layer of the combustion equipment are related to the content and composition of alkali metal element and/or alkaline earth metal element, combustible, non-combustible, or environmental temperature. When the content of alkali metal element and/or alkaline earth metal element in the combustion equipment is high, the destroy and rebuild of the surface layer of the combustion equipment is faster, resulting in a higher heat generation speed.

There will be a carbon-containing material formed on surface of combustion equipment as a result of adding alkali metal element and/or alkaline earth metal element into the combustible in this invention. According to need, the types and contents of alkali metal element and/or alkaline earth metal element added into the combustible can be manipulated to make the carbon-containing material layer have a function comprising lubrication, sealing, thermal conductivity, thermal insulation, high and low temperature resistance, wear resistance, thermal shock resistance, corrosion resistance, explosive combustion resistance, or surface defect repairment of combustion equipment. Therefore, the combustion equipment has a higher combustion temperature, faster combustion speed and more complete combustion, faster heating speed, lower friction resistance, higher temperature resistance of rotor and blade, higher power output of combustion equipment, longer mechanical usage life, lower working noise, smaller volume of combustion equipment. According to the theory proposed by Professor Dr. Yongheng ZHANG, the power output of combustion equipment can be fold increased than the prior arts.

Another important technical feature of the method for promoting the combustion of combustible, and enhancing power output and usage life of combustion equipment is that the exhaust gas of the first combustion equipment can be more efficiently utilized to heat the secondary combustion equipment. Due to the addition of alkali metal element and/or alkaline earth metal element into the combustible, the exhaust gas contains alkali metal element and/or alkaline earth metal element. The alkali metal element and/or alkaline earth metal element will destroy and rebuild the surface layer of the secondary combustion equipment, generating heat to heat the secondary combustion equipment. The secondary combustion equipment includes a boiler, industrial kiln, heating box or refrigeration device. The boiler drives a steam turbine, and the steam turbine drives the generator. Therefore, the energy conversion efficiency of combustible is further improved.

In a conclusion, the combustion of combustible and power output and usage life of combustion equipment are improved, different carbon-containing organic matters are fully used as the fuel, the volume of combustion equipment is reduced, the power output of combustion equipment is increased, the mechanical structure of combustion equipment is simplified, the combustion efficiency of combustible is increased, the combustion equipment starts and works efficiently, the reliability of combustion equipment is improved, by using the method provided by this invention.

### Advantageous Effects

The advantages of present invention include but are not limited to:
(1) The method provided by this invention can promote the combustion of all type of the combustible, such as carbon, resin, polyethylene plastic, gasoline, diesel, bio-diesel, bio-ethanol, bio-methanol, plant oil, animal oil, natural gas, liquefied petroleum gas, coal to gas, ethanol, methanol, toluene, methane, acetylene, ethane, ammonia, hydrogen, deuterium, tritium, sulfur, phosphorus, metal or mixtures of the aforementioned. The method is applicable to all kind of combustion equipment, such as gasoline engine, diesel engine, internal combustion engine, piston engine, turbofan engine, turbojet engine, rocket engine, nuclear fusion reactor, nuclear fission reactor, fuel cell, gas turbine, boiler, and thermoelectric converter. But the existing technology is only for limited several kinds of combustible and combustion equipment.
(2) This invention to add alkali metal element and/or alkaline earth metal element into the combustible, can not only improve the combustion efficiency of the combustible, but also control the combustion characteristics and combustion process by adjusting the combustion efficiency, combustion rate, combustion characteristics of the combustible. Through controlling the combustion characteristics, the noise and vibration of combustion process can be controlled. However, the existing technology cannot achieve this technical goal.
(3) This invention to add alkali metal element and/or alkaline earth metal element into the combustible, leads to the formation of a carbon-containing material layer on surface of the combustion equipment with various functions, (such as lubrication, wear resistance, thermal conductivity, thermal insulation, corrosion resistance, high and low temperature resistance, thermal shock resistance, etc.), and hence reduce the combustion noise, increase the combustion temperature, enhance the output power and the usage life of the combustion equipment. Moreover, the liquid cooling system of gasoline engines, diesel engines, gas piston engines, etc. can be omitted, so as to simplify the mechanical structure of the engine. The existing technology cannot achieve this technical goal.
(4) This invention to add alkali metal element and/or alkaline earth metal element into the combustible, leads to the increase of efficiency and combustion rate of the combustible, reduction of combustion equipment volume. For example, a power output of 1-liter gasoline or diesel engine is equivalent to an existing 2.5-liter gasoline or diesel engine, while a 50-centimeter diameter jet or rocket engine generates a thrust equivalent to an existing 1-meter diameter engine. As a result, the fuel consumption is greatly reduced and the usage life is extended. The existing technology cannot achieve this technical goal.
(5) This invention to add alkali metal element and/or alkaline earth metal element into the combustible can reduce the noise and vibration of the combustion equipment during the combustion process, while the existing technology cannot control the noise and vibration during the combustion process.
(6) This invention to add alkali metal element and/or alkaline earth metal element into the combustible can increase the combustion rate and combustion temperature, thereby saving a large amount of fuel, (usually between 20% and 40% for current gasoline engines). The existing technology can only have a small combustion promoting effect on one type of fuel, and the fuel saving is normally below 10wt%.
(7) This invention to add alkali metal element and/or alkaline earth metal element into the combustible can make the combustible to be lighted easily at high altitude area, high air area, or universal space, and increase the combustion efficiency of the combustible, and greatly increase the power output and save the fuel. But the existing technology cannot achieve this technical goal.
(8) This invention to add alkali metal element and/or alkaline earth metal element into the combustible can make the combustion equipment start normally and work efficiently. For example, all kind of combustion equipment start normally and work efficiently at a temperature from -250°C to 2500°C in space. The existing technology cannot achieve this technical goal.
(9) This invention to add alkali metal element and/or alkaline earth metal element into the combustible can improve the combustion efficiency and thermal efficiency of fuels such as bio-diesel, bio-ethanol, bio-methanol, plant oil, animal oil, plant oil, plant-derived fuel making them suitable for various combustion equipment such as piston engines, gas turbines, jet engines, or rocket engines. But the existing technology cannot achieve this technical goal.
(10) The additive to promote the combustion of combustible is non-toxic, harmless, cost-effective, and recyclable.
(11) The effect of exhaust gas of combustion equipment using prior arts to heat other heating equipment is poor, and the exhaust gas cannot be utilized or well utilized. In this invention, the alkali metal element and/or alkaline earth metal element is added into the combustible enabling the exhaust gas of the first combustion equipment generating more heat for heating the secondary combustion equipment, thereby further improving the combustion efficiency and energy conversion efficiency of the fuel. But the existing technology cannot achieve this technical goal.
(12) The technology disclosed in this invention can enable mixed fuel for various combustion equipment. The mixed fuel comprises several of diesel, gasoline, bio-diesel, bio-ethanol, ethanol, methane, ammonia, animal oil and plant oil, polymer-derived or plant-derived carbon containing organic matter. Therefore, various kinds of fuels are fully utilized and their combustion efficiency is improved. But the existing technology cannot achieve this technical goal.
(13) The fuel provided by this invention can initiate nuclear fusion reaction or nuclear fission reaction, and keep the nuclear fusion or nuclear fission proceed and be controllable, so the nuclear fusion or nuclear fission can be utilized and commercialized. But the existing technology cannot achieve this technical goal.
(14) This invention provides the nuclear fusion reactor or nuclear fission reactor to make nuclear fusion or nuclear fission reaction be controllable. But the existing technology cannot achieve this technical goal.
(15) This invention provides the fuel and engine enabling ammonia mixed fuel engine and hydrogen mixed fuel engine start and work normally. But the existing technology cannot achieve this goal.
(16) This invention can make fuel cell having higher efficiency. But the existing technology cannot achieve this technical goal.
(17) This invention provides the combustion equipment, for example diesel engine, without liquid cooling system, or forced lubrication system. But the existing technology cannot achieve this technical goal.
(18) This invention provides the fuel and combustion equipment to prevent explosive combustion, so as to make combustion process safer. But the existing technology cannot achieve this technical goal.
(19) This invention can greatly enhance the mechanical reliability of combustion equipment, so as to enhance its usage life. But the existing technology cannot achieve this technical goal.

### Industrial applications

The industrial application of this invention includes but not limited to the followings. the fuel to enable the combustion equipment with higher combustion efficiency and higher power output and longer usage life;
the fuel to prevent explosive combustion;
the combustion process to be safer and reliable;
the combustion equipment using mixed fuel;
the combustion equipment with a compact structure, higher power, longer usage life and safer;
the better control of combustion equipment;
the combustion equipment to be lighted, start and work at any environment;
the combustion chamber of combustion equipment without liquid cooling system, or without forced lubrication system;
the reduction of toxic emission;
the realization and control of nuclear fusion and nuclear fission reaction.

### Detailed Description of Embodiments

The present invention provides the method to promote the combustion of the combustible, enhance the power output and usage life of combustion equipment by adding alkali metal element and/or alkaline earth metal element into the combustible. The state of combustible comprises one or more of gas, liquid, and solid. The alkali metal element comprises one or more of Li, Na, K, Rb, Cs, and Fr, and the alkaline earth metal element comprises one or more of Be, Mg, Ca, Sr, Ba, and Ra.

Different from prior technology, this invention is applicable to all combustible, for example, one or more of carbon, carbon-containing organic matter, carbon dioxide, ammonia, hydrogen, sulfur, phosphorus, and metal. The carbon comprises carbon power. The carbon-containing organic matter preferably comprises one or more of all carbon-containing organic matter, such as resin, polyethylene plastic, gasoline, diesel, kerosene, bio-diesel, vegetable oil, animal oil, bio-ethanol, bio-methanol, natural gas, aviation kerosene, liquefied petroleum gas, coal to gas, ethanol, methanol, toluene, acetylene, methane, ethane, and polymer-derived or plant-derived carbon-containing organic matter.

In this invention, the state of alkali metal element and/or alkaline earth metal element can be any state, preferred one or more of atom, ion, and plasma.

In some embodiments, the alkali metal element and/or alkaline earth metal element is added by the matter containing alkali metal element and/or alkaline earth metal element. The matter containing alkali metal element and/or alkaline earth metal element comprise one or more of plasma, elementary substance, alloy, compound or composition of alkali metal element or alkaline earth metal element. Preferred, it is added in a form comprising one or more of plasma, elementary substance, alloy, compound or composition. The matter containing alkali metal element and/or alkaline earth metal element can be any state, preferably comprising plasma, gas, liquid, or solid. The compound or composition comprises one or more of all organic compounds or inorganic compounds.

In some embodiments, when the alkali metal element is added by an elementary substance, the alkali metal element comprises at least one of Li, Na, K, Rb, Cs, or Fr element. When the alkali metal element is added by an alloy, the alloy can be any type of alloy containing alkali metal elements, for example lithium aluminum alloy, calcium lithium silicon alloy, lithium calcium alloy, calcium magnesium lithium alloy, iron nickel magnesium lithium carbon alloy, titanium lithium alloy, and titanium magnesium lithium alloy. When the alkali metal element is added by a compound, the compound comprises one or more of all compounds of the alkali metal element. The compound comprises organic compound, or inorganic compound, for example, organic acid salts, inorganic acid salts, oxides, bases, alcohols, phenols, acetate salts, oxalates, citrate salts, hydrochloride salts, sulfates, carbonates, aluminosilicates, phosphates, and hydroxides. It should be noted that the alkali metal elements in these compounds are necessary elements for generating plasma to initiate combustion. The other ions or components that make up these compounds can affect the temperature required to ignite combustion. The choice of compound to be added is determined by the type of combustion equipment and the type of the combustible. For example, the piston engine allows for a lower combustion temperature, the compounds that are easily decomposed and ionized, such as acetate, oxalate, citrate, or chloride are added. For the combustion equipment that allows higher combustion temperature, such as turbines, jet engines, and rocket engines, an additional quantity of compounds with higher thermal decomposition temperatures and lower ionization rates, such as phosphates, aluminosilicates, and hydroxides, needs to be added to ensure a sustained supply of alkali metal element and/or alkaline earth metal element inside the combustion chamber.

In some embodiments, the compound containing alkali metal element comprises at least one of sodium hydroxide, potassium hydroxide, lithium acetate, potassium acetate, and sodium acetate. When the alkali metal elements are added by a mixture, the mixture is lithium acetate and potassium acetate, or potassium acetate and potassium hydroxide, or sodium acetate and sodium hydroxide, or potassium acetate and sodium hydroxide, or potassium acetate and sodium acetate and lithium acetate. The alkali metal element can also be mixed with alkaline earth metal elements to get a mixture followed by adding it into the combustible. The mixture examples are magnesium chloride and potassium hydroxide, or magnesium chloride and sodium hydroxide, or magnesium chloride and potassium acetate, or magnesium chloride and sodium acetate, or calcium chloride and potassium acetate and lithium acetate and sodium acetate.

In some embodiments, when the alkaline earth metal element is added by an elementary substance, the element comprises at least one of Be, Mg, Ca, Sr, Ba, or Ra. When the alkaline earth metal element is added by an alloy, the alloy can be any type of alloy containing alkaline earth metal element, for example, magnesium aluminum alloy, calcium silicon alloy, lithium calcium alloy, calcium magnesium lithium alloy, iron calcium magnesium carbon, iron nickel calcium carbon alloy, titanium magnesium lithium alloy. When the alkaline earth metal element is added by a compound, the compound comprises one or more of all alkaline earth metal compounds. The compound comprises organic compounds, inorganic compounds or oxides, specifically such as organic acid salts, inorganic acid salts, or bases. More specifically, the compound comprises one or more of alcohols, phenols, acetate salts, oxalates, citrate salts, hydrochloride salts, sulfates, carbonates, aluminosilicates, phosphates, and hydroxides. It should be noted that the alkaline earth metal elements in these compounds are necessary elements for generating plasma. The other ions or components that make up these compounds can affect the temperature required to ignite the combustion. The selection of compounds to be added depends on the type of combustion equipment and the type of combustible. The principle of adding alkaline metal elements is the same as the one mentioned earlier for alkali metal elements. In some embodiments, the alkaline earth metal element is added by organic acid salt, inorganic acid salt, or base, for example, acetate or hydrochloride. In some embodiments, the compound containing alkaline earth metal element is magnesium chloride, magnesium acetate, or calcium chloride. When the alkaline earth metal element is added by a mixture, the example of the mixture is magnesium chloride and magnesium acetate. The alkali metal element and alkaline earth metal element can be simultaneously added into the combustible. For example, the magnesium chloride and potassium acetate, magnesium chloride and potassium hydroxide, calcium chloride and potassium acetate, or calcium chloride and lithium acetate and sodium acetate is added into the combustible. The specific addition quantity depends on the combustion equipment and combustible. It should be emphasized that the alkali metal element and alkaline earth metal element can be also added into the combustible by an alloy, such as aluminum magnesium lithium alloy, aluminum calcium lithium alloy, iron magnesium carbon alloy, iron nickel calcium magnesium carbon alloy, titanium lithium alloy, or titanium magnesium lithium alloy. These alloys are also used to manufacture the combustion equipment, particularly suitable for manufacturing the combustion chambers and their components such as cylinder liner, piston, rotor and blade.

In some embodiments, the addition amount of alkali metal element and/or alkaline earth metal element is preferably from Owt% to 10000.9999999999999999wt% of the mass of the combustible, and not to be 0. In some embodiments, the addition amount is from Owt% to 90.9999999999999999wt%. In this invention, the alkali metal element and/or alkaline earth metal element reacts with carbon element forming a new carbon-containing material, or forming the plasma to ignite the combustion and make the combustion process to continue. In the meantime, the alkali metal element and/or alkaline earth metal element destroys and rebuilds the carbon-containing material layer on surface of the combustion equipment generating the heat to heat the combustion equipment, so as to further promote the plasma formation. This is to say that the formation of plasma and heat up of combustion equipment is promoted each other until the destroy and rebuild of the carbon-containing material layer reaches an equilibrium. Then, the temperature of the combustion equipment also reaches an equilibrium.

In this invention, the combustion equipment comprises all kind combustion equipment. The combustion equipment can start and work efficiently at any environment and output higher power and has a longer usage life and higher mechanical reliability.

In some embodiments, the combustion equipment preferably comprises one or more of first combustion equipment and secondary combustion equipment heated by exhaust gas from first combustion equipment. The first combustion equipment preferably comprises one or more of gasoline engine, diesel engine, internal combustion engine, ammonia mixed fuel engine, hydrogen mixed fuel engine, mixed fuel engine, piston engine, turbofan engine, turbojet engine, rocket engine, mixed fuel gas turbine, gas turbine, boiler, nuclear fusion reactor, nuclear fission reactor, fuel cell, warmer, oven, thermoelectric converter, or combustion refrigerator. The secondary combustion equipment heated by exhaust gas of first combustion equipment comprises boiler, industrial kiln, refrigerator, thermoelectric converter or combustion refrigerator. The boiler comprises steam boiler, or hot water boiler.

In this invention, the addition of alkali metal element and/or alkaline earth metal element can make the carbon layer of combustion surface be destroyed and rebuilt constantly to generate the heat to heat the combustion equipment. Particularly important, the exhaust gas of first combustion equipment contains a high concentration of alkali metal element and/or alkaline earth metal element and a low concentration of carbon-containing organic matter. This kind of exhaust gas can easily destroy the carbon layer of secondary combustion equipment producing plasma to heat the combustion equipment. Therefore, the thermal efficiency or energy conversion efficiency of fuel is further improved.

In this invention, there will be a carbon-containing material formed on the surface of combustion equipment during the combustion process of the combustible containing alkali metal element and/or alkaline earth metal element. The carbon-containing material contains alkali metal element and/or alkaline earth metal element with a thickness from 0.1 nm to 1 mm. The carbon-containing material has at least one of functions comprising lubrication, wear resistance, sealing, thermal conductivity, thermal insulation, high and low temperature resistance, thermal shock resistance, corrosive resistance, explosive combustion resistance and surface defect repairment of combustion equipment. Therefore, the combustion equipment can be without a liquid cooling system, or without external forced lubrication system.

Particularly important, the alkali metal element and/or alkaline earth metal element can be added into the deuterium and tritium to initiate hydrogen nuclear fusion and keep the nuclear fusion process continue and be under control. The hydrogen nuclear fusion is initiated by plasma and there need more alkali metal element and/or alkaline earth metal element during nuclear fusion process.

In some embodiments, the addition amount of the alkali metal element and/or alkaline earth metal element into deuterium and tritium is 0.000000000000001wt%-1000wt% of mass of deuterium and tritium. Similarly, the nuclear fusion of metal needs to make the metal become into a plasma by alkali metal element and/or alkaline earth metal element, so as to realize the reaction among nucleus. In some embodiments, the content of alkali metal element and/or alkaline earth metal element in fuel of nuclear fusion is 0.0001wt%-100wt%. Based on the same principle, the nuclear fission of nonradioactive metal also needs to become into a plasma of super high temperature using alkali metal element and/or alkaline earth metal element, so as to realize the fission of metal nucleus into new metal and new metal-carbon-containing material composite. The inventor wants to explain specifically that the nuclear fusion or nuclear fission must involve the carbon-containing organic matter to make fusion material or fission material become into the plasma. Only by using the fuel and combustion equipment disclosed by the method of this invention, the plasma of superhigh temperature can be produced, so as to realize the nuclear fusion reaction or nuclear fission reaction and control the process of nuclear fusion reaction or nuclear fission reaction.

In some embodiments, the carbon-containing organic matter and alkali metal element and/or alkaline earth metal element is added into ammonia or hydrogen to produce the fuel. The addition amount of alkali metal element and/or alkaline earth metal element is 0.0001wt%-10000wt% mass of ammonia or hydrogen. In this invention, the approach to add alkali metal element and/or alkaline earth metal element comprises at least one of approach 1, 2, 3 and 4.

In some embodiments, the approach to add the alkali metal element and/or alkaline earth metal element is added into the combustible comprises approach 1. The approach 1 comprises adding the matter containing alkali metal element and/or alkaline earth metal element into the combustible by mixing, ball milling, crushing, melting, electric sparkling, or plasmazing, or adding the matter containing alkali metal element and/or alkaline earth metal element into noncombustible followed by adding the mixture into the combustible. The matter containing alkali metal element and/or alkaline earth metal element comprises one or more of elementary substance, alloy, compound and composition, and it will not be explained later. The mixing temperature preferably is 0-500°C, or lower than -100°C. For example, for cryogenic liquid such as liquid oxygen, liquid hydrogen, liquefied natural gas and liquid methane, etc need mixing at low temperature, normally below -100°C. The approach 1 is applicable to the combustible of any matter state. The noncombustible comprises one or more of all kind noncombustible. The example of the noncombustible is H₂O, N₂, O₂, NO, CO₂, Fe₂O₃, or SiO₂.

In some embodiments, the approach to add the matter containing alkali metal element and/or alkaline earth metal element into the combustible comprises approach 2. The approach 2 comprises dissolving the matter containing alkali metal element and/or alkaline earth metal element into the combustible. The approach 2 is applicable to all not-gaseous combustible.

In some embodiments, the approach to add the matter containing alkali metal element and/or alkaline earth metal element comprises approach 3. The approach 3 comprises mixing the matter containing alkali metal element and/or alkaline earth metal element with a solvent to obtain a solution or suspension or paste, followed by adding them into the combustible. The solvent comprises at least one of inorganic solvent or organic solvent. The examples of the inorganic solvents are water and organic acid solutions. The examples of the organic solvent are formic acid, alcohols, aromatic hydrocarbons, aliphatic hydrocarbons, alicyclic hydrocarbons, or halogenated hydrocarbons. In a embodiments of the present invention, the organic solvent is ethanol.

In some embodiments, the approach to add the matter containing alkali metal element and/or alkaline earth metal element into the combustible comprises approach 4. The approach 4 comprises producing the combustion chamber, component of combustion chamber, tank of oil or fuel or combustion supporting material, filter, or pipeline of combustion equipment with the material containing alkali metal element and/or alkaline earth metal element. This kind of combustion equipment can start and work efficiently at any environment and output higher power and has longer usage life.

The material containing alkali metal element and/or alkaline earth metal element comprises one or more of polymer, ceramics or metal. The polymer preferably comprises rubber. The metal comprises elementary substance and/or alloy. When the combustible or noncombustible contacts with these materials, they will react with alkali metal, alkaline earth metal, alkali metal compound, alkaline earth metal compound, metal or alloy forming the compound containing alkali metal element and/or alkaline earth metal element, which is then mixed with combustible and/or combustion supporting material. The combustion equipment and its component comprise combustion chamber, cylinder liner, nozzle, spark plug, piston, connecting rod, rotor or blade. The content of alkali metal element and/or alkaline earth metal element of the material containing alkali metal element and/or alkaline earth metal element is preferably 0.0000000001wt%-99.99wt%. The content of alkali metal element and/or alkaline earth metal element of alloy is preferably 0.0000000001wt%-99.99wt%.

In some embodiments, the part of combustion equipment is produced with through-hole, dent, or protrusion, so as to form different matters containing alkali metal element and/or alkaline earth metal element. During combustion process, these positions release different matters containing alkali metal element and/or alkaline earth metal element in different spaces of combustion chamber to prevent the deletion or content fluctuation of alkali metal element and/or alkaline earth metal element, so as to adjust the combustion state of combustion chamber.

The maximum cross-sectional area of the orifice of through-hole, orifice of dent or base of protrusion of the part of combustion equipment is from 0.01 square nanometers to 1 square meters. The depth of dent or height of protrusion is from 0.1 nm to 100 mm. The dent or protrusion is any geometry. The part comprises one or more of combustion chamber or its component.

In some embodiments, the part or some parts of combustion equipment are made of the material containing alkali metal element and/or alkaline earth metal element. The content of alkali metal element and/or alkaline earth metal element in the material containing alkali metal element and/or alkaline earth metal element is Owt%-99.990000000000wt%, and not to be 0. The material containing alkali metal element and/or alkaline earth metal element comprises polymer, metal or ceramics. The combustion equipment comprises any kind of combustion equipment. This kind of combustion equipment can promote the combustion of combustible, improve the power output and prolong the usage life, and has high mechanical reliability.

This invention also provides a piston engine. The piston engine comprises a liquid cooling system or does not comprise a liquid cooling system. The fuel of the piston engine is the fuel disclosed by this invention. The combustible of the fuel comprises one or more of gasoline, diesel, bio-diesel, plant oil, animal oil, bio-ethanol, bio-methane, ethanol, methanol, hydrogen, ammonia, natural gas, acetylene, methane, or liquefied petroleum gas, polymer-based and plant-based carbon-containing organic matter.

In some embodiments, the inner surface of cylinder of piston engine has dent, or the outer surface of cylinder of piston engine has dent or protrusion. The dent or protrusion is any shape and structure. There is protrusion or is not protrusion in the dent. The arrangement of the dent or protrusion is regular or non-regular. The surface area of orifice of dent or base of protrusion is from 0.01 square nanometers to 0.03 square nanometers. The depth of dent or height of protrusion is from 0.1 nm to 100 mm. In some embodiment, the inner surface of cylinder has groove, and/or blind hole. The outer surface of cylinder has groove, blind hole or protrusion. The width of groove or protrusion, or diameter of blind hole is preferably from 0.1 nm to 100 mm. The depth of groove or blind hole is from 0.1 nm to 50 mm. The height of protrusion is preferably from 0.1 nm to 100 mm, or preferably from 1 nm to 20 mm. The groove or protrusion is any geometry. The arrangement pattern of groove or protrusion or blind hole is regular or irregular. The groove or blind hole is prefilled or is filled during combustion process with carbon-containing material containing alkali metal element and/or alkaline earth metal element. The filled carbon-containing material containing alkali metal element and/or alkaline earth metal element in groove or blind hole acts as a storage of alkali metal element and/or alkaline earth metal element, and improve at least one of the characteristics comprising sealing, thermal conductivity, lubrication, wear resistance, explosive combustion resistance, high and low temperature resistance and thermal shock resistance.

In some embodiments, the piston engine disclosed by this invention can be without liquid cooling system or without external forced lubrication system. Therefore, the structure of piston engine is further simplified to enhance its reliability.

In some embodiments, because this invention allows the cylinder to have more air or other kind of gas, the piston engine can equip with a compressed gas intaking system to increase the gas amount and cylinder pressure during combustion process to further improve the power output of piston engine.

In this invention, the piston engine has a spark plug ignition system or does not have a spark plug ignition system. The fuel of the piston engine comprises one or more of gasoline, diesel, bio-diesel plant oil, animal oil, bio-ethanol, bio-methanol, ethanol, methane, ammonia, hydrogen, natural gas, acetylene, methane, liquefied petroleum gas, polymer-based carbon-containing organic matter and plant-based carbon-containing organic matter.

This invention also provides a fuel which can enhance power output and usage life of combustion equipment by adding alkali metal element and/or alkaline earth metal element into combustible. In some embodiments, the content of alkali metal element and/or alkaline earth metal element in the fuel is 0wr%-10000.9999999999999999wt%, and not to be 0. In some embodiments, the content of alkali metal element and/or alkaline earth metal element in the fuel is 0wr%-90.9999999999999999wt%, and not to be 0. The approach to add alkali metal element and/or alkaline earth metal element into the fuel is the same as descried above, and it is not explained again here.

This invention also provides a high-efficiency fuel energy conversion system. It comprises the combustion equipment and fuel. The fuel is the fuel described above. The combustion equipment can be any combustion equipment, particularly the combustion equipment described above, preferably comprising one or more first combustion equipment and secondary combustion equipment. The kinds of first and secondary combustion equipment are not explained again. In some embodiments, the combustion equipment can be thermoelectric converter, nuclear fusion reactor, nuclear fission reactor, engine, or the heating equipment heated by exhaust gas of engine. The heating equipment preferably comprises boiler, industrial kiln, air heater, oven or refrigerator. The boiler comprises steam boiler or hot water boiler. The equipment powered by engine comprises electrical generator, vehicle, ship or train. The steam boiler powers steam turbine, and the steam turbine powers the electrical generator. The heating equipment utilizes the alkali metal element and/or alkaline earth metal element to destroy and rebuild the surface layer to generate heat to heat up.

In some embodiments, the high-efficiency fuel energy conversion system preferably comprises other energy conversion system connected to combustion equipment. The other energy conversion equipment preferably comprises refrigeration equipment, hot-water boiler, steam boiler, industrial kiln, industrial oven, thermoelectric converter, or electrical generator powered by steam boiler.

The high-efficiency fuel energy conversion system can start and work efficiently and explosive combustion prohibited, output higher power, have longer usage life and higher mechanical reliability.

The following will give a clear and complete description of the technical solution with examples. Obviously, these examples are only a portion of the embodiments of the present invention. Based on the embodiments of this invention, all other examples obtained by ordinary technicians in the art without creative labor fall within the protection scope of this invention.

### Example 1

2 g of lithium acetate dihydrate was dissolved into 500 ml of anhydrous ethanol to form a lithium acetate ethanol solution. 100 ml of lithium acetate ethanol solution were measured and injected into the car fuel tank. Then, 25 liters of No.92 gasoline were injected into the car fuel tank. Then, the car was tested by driving. It was found that the fuel consumption per 100 km decreased from 12 liters to 10 liters. Due to the generation of more plasma during the combustion process, the combustion is more rapid and complete resulting a higher power output. During combustion process, a carbon-containing material layer with good lubrication, thermal insulation and sealing effects is generated on the surface of the cylinder, which increases engine power output, reduces fuel consumption by 17%, and reduces engine noise. (Test conditions: The car's engine is 2.5-liter naturally aspirated, with a driving distance of about 133000 km. It was manufactured in 2010. The car is driven on urban road six times a day, with an average driving distance of about 5 km per time and an average speed of about 25 km per hour.).

### Example 2

5 g of magnesium chloride hexahydrate were dissolved into 500 ml of ethanol to obtain an ethanol solution of magnesium chloride. 100 ml of magnesium chloride ethanol solution were measured and injected into the car fuel tank. Then, 25 liters of No.92 gasoline was injected into fuel tank. Then, the car was tested by driving. It was found that the fuel consumption per 100 km decreased from 12 liters to 10 liters, saving 20% of gasoline. The testing conditions are the same as in Example 1.

### Example 3

5 g of potassium acetate were dissolved into 500 ml of ethanol to obtain a potassium acetate ethanol solution. 100 ml of potassium acetate ethanol solution were injected into the car fuel tank, followed by adding 25 liters of No.92 gasoline into the fuel tank. Then, the car was tested by driving. It was found that the fuel consumption per 100 km decreased from 12 liters to 9.3 liters, and the fuel consumption decreased 22.5%. Testing conditions are the same as Example 1.

### Example 4

(1) Dissolve 2 g of sodium hydroxide into 500 ml of ethanol to prepare a solution.
(2) Dissolve 5 g of potassium hydroxide into 500 ml of ethanol to prepare a solution.
(3) Dissolve 5 g of anhydrous potassium acetate into 500 ml of ethanol to prepare a solution.
(4) Dissolve 2 g of anhydrous sodium acetate into 500 ml of ethanol to prepare a solution.
(5) Dissolve 5 g of magnesium chloride hexahydrate into 500 ml of ethanol to prepare a solution.
(6) Dissolve 2 g of lithium acetate dihydrate into 500 ml of ethanol to prepare a solution.
(7) Dissolve 2 g of magnesium acetate tetrahydrate into 500 ml of ethanol to prepare a solution.

A certain amount of the above solution was added into 10 liters of gasoline, as shown in Table 1. Then the car described in Example 1 was driven on the urban elevated road at an average speed of 58 km per hour until 10 liters of gasoline are depleted. The driving distance, fuel consumption, and fuel efficiency of the car are shown in Table 1. When alkali metal element and/or alkaline earth element is not added into gasoline, the fuel consumption of the car is 11.5 liters per 100 km (30 km/h), 8.5 liters per 100 km (58 km/h), and 8.3 liters per 100 km (90 km/h). During driving test, the cooling fan of the coolant does not rotate. It should be noted that in this example, the gasoline cannot be used up every time. There are still about 3 liters of gasoline left in the fuel tank. Therefore, it is inevitable that there will be a mixture of remaining gasoline and newly added gasoline in each test. The results are that the content of various compounds in the fuel tank is not exactly the content listed in the Table 1. This result also indicates that the combustion promotion technology of present invention has strong practicality.

**Table 1. Driving distance, fuel consumption, percentage of fuel saved after adding different solutions into the car fuel**

| No. | Compound and quantity/10 liters gasoline | Driving distance and speed | Fuel consumption (liter/100 km) | Fuel saved (liter/100 km) | Percentage of fuel saved (Fuel saved/original fuel consumption)x100 % |
|---|---|---|---|---|---|
| 1 | 80 ml KOH | 165 km, 58 km/h | 6.06 | 2.44 | 29% |
| 2 | 5 ml of MgCl₂ and 20 ml of anhydrous potassium acetate | 160 km, 90 km/h | 6.25 | 2.05 | 25% |
| 3 | 40 ml of anhydrous potassium acetate | 173 km, 58 km/h | 5.78 | 2.72 | 32% |
| 4 | 25 ml of MgCl₂ and 50 ml anhydrous potassium acetate | 171 km, 58 km/h | 5.84 | 2.66 | 31 |
| 5 | 100 ml of MgCl₂ | 157 km, 90 km/h | 6.37 | 1.93 | 23% |
| 6 | 50 ml of MgCl₂ | 180 km, 58 km/h | 5.56 | 2.94 | 35% |
| 7 | 50 ml of MgCl₂ and 50 ml of anhydrous potassium acetate | 171 km, 90 km/h | 5.85 | 2.45 | 30% |
| 8 | 100 ml of anhydrous potassium acetate | 120 km, 30 km/h | 8.33 | 3.17 | 28% |
| 9 | 100 ml of anhydrous potassium acetate | 160 km, 90 km/h | 6.25 | 2.05 | 25% |
| 10 | 80 ml of NaOH | 160 km, 58 km/h | 6.25 | 2.25 | 26% |
| 11 | 40 ml of NaOH and 40 ml of anhydrous sodium acetate | 163 km, 58 km/h | 6.13 | 2.37 | 28% |
| 12 | 40 ml of NaOH and 80 ml of anhydrous sodium acetate | 178 km, 58 km/h | 5.61 | 2.89 | 34% |
| 13 | 40 ml of NaOH and 160 ml of anhydrous sodium acetate | 150 km, 58 km/h | 6.67 | 1.83 | 21% |
| 14 | 80 ml of lithium acetate dihydrate | 140 km, 58 km/h | 7.14 | 1.36 | 16% |
| 15 | 20 ml of lithium acetate dihydrate and 20 ml of anhydrous sodium acetate and 25 ml of anhydrous potassium acetate | 150 km, 58 km/h | 6.66 | 1.84 | 22% |
| 16 | 25 ml of CaCl₂ | 158 km, 58 km/h | 6.33 | 2.17 | 26% |
| 17 | 80 ml of magnesium acetate tetrahydrate | 150 km, 58 km/h | 6.66 | 1.84 | 22% |

### Example 5

To verify the application field of the present invention in promoting the combustion of combustible materials. A set of experiments involves adding 80 ml of sodium acetate solution from Example 5 to the fuel tank, then adding 1 liter of ethanol, 1 liter of methanol, and 8 liters of gasoline to the fuel tank, followed by a driving experiment. One experiment involves adding 40 ml of potassium acetate solution from Example 5 to the fuel tank, then adding 3 liters of ethanol and 7 liters of gasoline to the fuel tank, followed by a driving experiment. Another set of experiments involves adding 20 ml of potassium acetate solution and 20 ml of sodium acetate solution from Example 5 to the fuel tank, then adding 3 liters of methanol and 7 liters of gasoline to the fuel tank. The driving test results are shown in Table 2. The test results indicate that there is no significant decrease in thermal efficiency of ethanol and gasoline mixture, ethanol and methanol and gasoline mixture, or ethanol and methanol mixture compared to all gasoline fuels. One example is adding 1 liter peanut oil, and 9 liter gasoline and 80 ml potassium acetate solution to fuel tank. The test results demonstrate that the combustion promoting technology of the present invention is applicable to a variety of combustible materials.

**Table 2. Driving test results of gasoline mixed with ethanol or methanol**

| No. | Fuel composition | Driving distance (58 km/h) | Fuel consumption (liter/100 km) | Fuel saved (liter/100 km) | Fuel saved (liter/100 km) Percentage of fuel saved (fuel saved/original fuel consumption)x 100% |
|---|---|---|---|---|---|
| 1 | 1 liter ethanol, 1 liter methanol, 8 liter gasoline and 80 ml sodium acetate | 150 km , 58 km/h | 6.67 | 1.83 | 23% |
| 2 | 3 liter ethanol, 7 liter gasoline and 40 ml potassium acetate | 158 km , 58 km/h | 6.33 | 2.17 | 26% |
| 3 | 3 liter methanol, 7 liter gasoline, 20 ml potassium acetate solution and 20 ml sodium acetate | 155 km , 58 km/h | 6.45 | 2.05 | 24% |
| 4 | 1 liter peanut oil, 9 liter gasoline, 80 ml potassium acetate | 150 km | 6.67 | 1.83 | 23% |

### Example 6

The white printing paper was soaked in the potassium acetate solution of Example 5, and then dried under sunlight for two hours. Then, a small piece of the printing paper soaked or not-soaked in potassium acetate solution was separately put on a stainless steel discs. Then, the temperature of the stainless steel discs (with a thickness of 4 mm) was adjusted to 150 °C, 170 °C, and 203 °C by electric furnace The ignition times of the printing paper are measured. The test results, shown in Table 3, clearly demonstrate that potassium acetate can promote and keep the combustion of printing paper (resulting in open flames).

**Table 3. Combustion temperature of white printing paper smeared or not smeared with potassium acetate solution**

| Sample | Time to ignition at 150°C | Time to ignition at 170°C | Time to ignition at 203°C |
|---|---|---|---|
| With immersed potassium | Not ignition in 60 seconds | Not ignition in 60 seconds | 11 seconds |
| Without immersed potassium | Not ignition in 60 seconds | Not ignition in 60 seconds | 3 seconds |

The above are only examples. It should be point out that there are possibilities to make improvements based on the principle of this invention. All these improvements are within the protection scope of this invention.

## Claims

1. A method to promote combustion of combustible and enhance power output and usage life of combustion equipment, **characterized by** adding alkali metal element and/or alkaline earth metal element into combustible; wherein the matter state of the combustible comprises at least one of gas, liquid and solid, the alkali metal element comprises one or more of Li, Na, K, Rb, Cs and Fr, and the alkaline earth metal element comprises one or more of Be, Mg, Ca, Sr, Ba and Ra.

2. The method of claim 1, wherein the combustible comprises one or more of all combustibles.

3. The method of claim 2, wherein the combustible comprises one or more of carbon, carbon-containing organic matter, ammonia, hydrogen, deuterium, tritium, sulfur, phosphorus or metals.

4. The method of claim 1, wherein the alkali metal element and/or alkaline earth metal element is added into the combustible by a form comprising at least one of atom, ion and plasma.

5. The method of claim 1, wherein the alkali metal element and/or alkaline earth metal element is added into the combustible by a form of any matter containing alkali metal element and/or alkaline earth metal element.

6. The method of claim 5, wherein the matter containing alkali metal element and/or alkaline earth metal element comprises one or more of all elementary substance, alloy, compound or composition containing alkali metal element and/or alkaline earth metal element, and the matter state of the matter containing alkali metal element and/or alkaline earth metal element comprises gas, liquid, solid or plasma.

7. The method of claim 1, wherein an addition amount of alkali metal element and/or alkaline earth metal element is 0wt%-100000.9999999999999999wt% of mass of the combustible, and not to be 0.

8. The method of claim 7, wherein the addition amount of alkali metal element and/or alkaline earth metal element is 0wt%-98.9999999999999999wt% of mass of the combustible, and not to be 0.

9. The method of claim 1, wherein the approach to add alkali metal element and/or alkaline earth metal element into the combustible by an approach comprising at least one of approach 1, 2, 3 or 4:
the approach 1 comprising: to add the matter containing alkali metal element and/or alkaline earth metal element into the combustible by mixing, ball milling, crushing, melting, electrical sparking or plasmazing, or to mix the matter containing alkali metal element and/or alkaline earth metal element with noncombustible followed by adding it into the combustible;
the approach 2 comprising: to dissolve the matter containing alkali metal element and/or alkaline earth metal element into the combustible;
the approach 3 comprising: to dissolve the matter containing alkali metal element and/or alkaline earth metal element into a solvent to obtain a solution or suspension or paste followed by adding it into the combustible;
the approach 4 comprising: to add the matter containing alkali metal element and/or alkaline earth metal element into part of combustion equipment; wherein the matter containing alkali metal element and/or alkaline earth metal element react with the combustible or noncombustible producing the matter containing alkali metal element and/or alkaline earth metal element, which is then added into the combustible; wherein the combustion equipment comprises all kinds of combustion equipment.

10. The method of claim 9, wherein the part of approach 4 is made of material containing alkali metal element and/or alkaline earth metal element; the material containing alkali metal element and/or alkaline earth metal element comprises one or more of polymer, ceramics or metal, the content of alkali metal element and/or alkaline earth metal element in the material containing alkali metal element and/or alkaline earth metal element is 0wt%-99.9900000000000wt%, but not to be 0, the part comprises one or more of combustion chamber, piston, connecting rod, cylinder, spray nozzle, spark plug, rotor, blade, nut, bolt inside combustion chamber, tank or pipeline of oil for combustion chamber, tank or pipeline of fuel, tank or pipeline of combustion supporting substance or filter.

11. The method of claim 9, in approach 4, the combustion chamber, or component of the combustion chamber, tank or pipeline of oil for combustion chamber or fuel or combustion supporting substance, or filter is made of material containing alkali metal element and/or alkaline earth metal element; the combustion chamber or component of combustion chamber comprises combustion chamber, piston, connecting rod, rotor, blade inside combustion chamber, the material containing alkali metal element and/or alkaline earth metal element comprises one or more of rubber, polymer-based composite, metal or alloy, the content of alkali metal element and/or alkaline earth metal element in the alloy is 0.00000000001wt%-99.99wt%.

12. The method of claim 1, wherein a surface of combustion chamber or part of combustion chamber of combustion equipment has through-hole, dent, or protrusion; the through-hole, dent, or protrusion is any geometry, the distribution of the through-hole, dent, or protrusion is randomly or regularly, wherein the through-hole or dent acts as a storage to add the matter containing alkali metal element and/or alkaline earth metal element into the combustible to avoid deficiency or content fluctuation of alkali metal element and/or alkaline earth metal element during combustion process, the through-hole, dent or protrusion adds different matters containing alkali metal element and/or alkaline earth metal element to adjust the matters containing alkali metal element and/or alkaline earth metal element with different chemical composition and structure in different spaces of combustion chamber, so as to further adjust the combustion state in different spaces to improve further the combustion efficiency.

13. The method of claim 1, wherein the matter containing alkali metal element and/or alkaline earth metal element, or the combustible containing the matter containing alkali metal element and/or alkaline earth metal element, or the noncombustible containing the matter containing alkali metal element and/or alkaline earth metal element is add to a fuel of combustion equipment.

14. The method of claim 1, wherein the combustion equipment comprises one or more of all combustion equipment.

15. The method of claim 14, wherein the combustion equipment comprises all internal combustion engine, external combustion engine, piston engine, turbofan engine, turbojet engine, rocket engine, gas turbine, boiler, nuclear fusion reactor, nuclear fission reactor, fuel cell, kitchen range, warmer, thermoelectric converter, refrigeration device or combustion refrigerator.

16. The method of claim 15, wherein the combustion equipment comprises one or more of first combustion equipment or secondary combustion equipment heated by exhaust gas of first combustion equipment, the first combustion equipment comprises one or more of gasoline engine, diesel engine, gas piston engine, jet engine, rocket engine, turbine, boiler and thermoelectric converter, the secondary combustion equipment comprises boiler, industrial kiln, thermoelectric converter, refrigeration device or combustion refrigerator.

17. A combustion equipment according to claim 1, wherein the part or some part of combustion equipment has a through-hole, dent, or protrusion; wherein there is or is not protrusion in dent, wherein the arrangement of dent or protrusion is regularly or irregularly, wherein the dent, protrusion or through-hole is any geometry, wherein the part comprises one or more of combustion chamber or parts inside combustion chamber.

18. The combustion equipment of claim 17, wherein the maximum cross-sectional area of orifice of through-hole or dent, or base of protrusion is from 0.01 square nanometers to 1 square meters, the depth of dent or height of protrusion is from 0.1 nm to 100 mm.

19. The combustion equipment of claim 17, wherein the part or some parts of the combustion equipment is made of material containing alkali metal element and/or alkaline earth metal element; the content of alkali metal element and/or alkaline earth metal element in the material containing alkali metal element and/or alkaline earth metal element is 0wt%-99.990000000000wt%, but not to be 0, the material containing alkali metal element and/or alkaline earth metal element comprises polymer, metal or ceramics, the part comprises one or more of combustion chamber or part inside combustion chamber, pipeline or tank of oil for combustion chamber, pipeline or tank of fuel, pipeline or tank of combustion supporting material, or filter.

20. A piston engine according to claim 1, wherein there is a dent on inner surface of cylinder; the dent has any geometry, there is or is not a protrusion in dent, the arrangement of dent is regularly or irregularly, the cross-sectional area of the orifice of dent is from 0.01 square nanometers to 0.03 square meters, the depth of dent is from 0.1 nm to 50 mm.

21. The piston engine of claim 20, wherein there is dent or protrusion on outer surface of cylinder, the cross-sectional area of orifice of dent, or the base of protrusion is from 0.01 nm to 0.03 square meters, the depth of dent or height of protrusion is from 0.1 nm to 50 mm.

22. The piston engine of claim 21, wherein there is a groove and/or blind hole on inner surface of cylinder, the width of groove or diameter of blind hole is from 0.001 µm to 10 mm, the depth of groove or blind hole is from 0.001 µm to 10 mm.

23. The piston engine of claim 20, wherein the part or some parts of the engine are made of material containing alkali metal element and/or alkaline earth metal element, the content of alkali metal element and/or alkaline earth metal element in the material containing alkali metal element and/or alkaline earth metal element is from Owt% to 99.990000000000wt%, wherein the material containing alkali metal element and/or alkaline earth metal element comprises polymer, metal or ceramics, the part comprises one or more of combustion chamber, parts inside combustion chamber, pipeline or tank of oil for combustion, pipeline or tank of fuel, pipeline or tank of combustion supporting material or filter.

24. The piston engine of claim 20, wherein the piston engine has or does not have a liquid cooling system, the combustible of the piston engine comprises one or more of gasoline, diesel, bio-diesel, plant oil, animal oil, bio-ethanol, bio-methanol, ethanol, methanol, ammonia, hydrogen, natural gas, acetylene, liquefied petroleum gas, polymer-derived carbon-containing organic matter, or plant-derived carbon-containing organic matter.

25. The piston engine of claim 20, wherein the piston engine has or does not have a liquid cooling system, the piston engine has a naturally aspirated system, or high-pressure intake system, the piston engine has or does not have an external forced lubrication system.

26. A fuel to promote combustion of combustible and enhance power output and usage life of combustion equipment according to claim 1, wherein the fuel comprises the combustible and alkali metal element and/or alkaline earth metal element, the content of alkali metal element and/or alkaline earth metal element is from Owt% to 100000.9999999999999999wt% of mass of the combustible, but not to be zero, the fuel enables the combustion equipment to start, to work efficiently, to be explosive combustion prohibited and to be mechanical reliable at any environment, the fuel is for one of all kind combustion equipment.

27. The fuel of claim 26, wherein the content of alkali metal element and/or alkaline earth metal element is from Owt% to 90.9999999999999999wt% of mass of the combustible, but not to be 0.

28. The fuel of claim 26 or 27, wherein the fuel comprises all kind of anti-explosive fuel, internal combustion fuel, external combustion fuel, piston engine fuel, mixed fuel engine fuel, mixed fuel, turbofan engine fuel, turbojet engine fuel, gas turbine fuel, boiler fuel, fuel cell fuel, nuclear fusion fuel, nuclear fission fuel, warmer fuel, oven fuel, thermoelectric converter, refrigeration device or combustion refrigerator.

29. A high-efficiency fuel energy conversion system according to claim 1, it comprises the fuel and combustion equipment; the fuel is any one of claim 26-28, the combustion equipment is any one of claim 14-16, or any one of claim 17-19, or any piston engine of claim 20-25.

30. The system of 29, wherein it comprises other energy conversion device connected with combustion equipment; the other energy conversion devices comprise refrigerator, hot water boiler, steam boiler, industrial kiln, industrial oven, thermoelectric converter or generator driven by steam boiler.
